

## UNITED STATES PATENT OFFICE

2,084,420

## MANUFACTURE OF PHOTOGRAPHIC PICTURES

Edith Weyde, Cologne-Niehl, Germany, assignor  
to Agfa Ansco Corporation, Binghamton, N. Y.,  
a corporation of New York

No Drawing. Application July 25, 1934, Serial  
No. 736,959. In Germany July 25, 1933

7 Claims. (Cl. 95—6)

My present invention relates to the manufacture of photographic pictures.

One of its objects is a process of producing photographic pictures. Further objects will be seen from the detailed specification following hereafter.

There are two fundamentally different processes for producing photographic pictures namely a printing process and a developing process. 10 In the printing process, the whole of the substance forming the picture is produced by the light itself, while in the developing process only a very small part of the sensitive material used is decomposed by the light and a latent, or very 15 faintly visible, image is obtained from which the full image is produced by a subsequent chemical process. For the developing process it has hitherto been possible to use only noble metal salts (Ag, Hg), in which the metal in question is 20 formed as a nucleus.

The present invention relates to a process of producing metal sulfide pictures by means of a developing method, wherein the sensitivity of the printing surface to light much exceeds that of 25 the surfaces used in the known developing processes and corresponds with that of the silver halide developing papers.

One method of producing metal sulfide pictures by a developing process is as follows:—Certain 30 heavy metal compounds of substances containing sulfur which in light are decomposed into the corresponding metal sulfides, are also affected in the same manner as by the light by different reagents, for instance, alkalies or acids, 35 and it has been found that this action is accelerated by small proportions of the metal sulfides in question. Accordingly, metal sulfide produced in traces by exposure to light acts as nuclei similarly to metallic silver in the ordinary 40 silver halide emulsions. Thus, for instance, the latent image of a bismuth-thiourea compound (obtainable by dissolving a bismuth-compound in thiourea solution) can be developed with caustic soda solution to bismuth-sulfide. For this process all metals are suitable which yield dark metal 45 sulfides, such as, for instance, lead, copper, bismuth, silver, mercury, thallium, molybdenum, tungsten, uranium, cobalt and nickel. As sulfur compounds in the sensitive layer and in the developer there may be used those which yield metal sulfides comparatively easily, such as, for example, thiourea and derivatives thereof, thioamides or thioacids. For developing there may be used alkaline baths which contain a substance 50 capable of converting the metal compound 55

into a sulfide; in certain cases, however, an acid development is possible. It is often not necessary to start with the metal compound of a sulfur compound. In most cases it is preferable to use a mixture of the sulfur compound and a metal combined otherwise than with the said sulfur compound. In this case it is advantageous that only a small proportion of the sulfur compound should be added to the sensitive layer itself (sufficient for the formation of metal sulfide nuclei), the main part being added to the developer. However, with certain compounds, such as complex compounds of cobalt, nickel or copper, it is unnecessary to add any sulfur compound to the sensitive layer since the sulfide nuclei can be formed in the developing bath. In these layers there are produced at the parts exposed to light ionizable metal compounds.

As sensitive material in this case there are suitable the various metal complex salts, for instance, of cobalt, nickel or copper with nitrates, oxalates, organic amines and phenolates which are so changed by light that compounds containing the metal in ionizable combination are produced. Many metal complexes react only relatively slowly with sulfur compounds, but very quickly when even only very small proportions of the metal ion in question are present. The metal ions are presumably converted very quickly into metal sulfide and act as nuclei for the further formation of sulfide from the complex compound. It is in this case advantageous not to use sodium sulfide as developer but a compound in which the reactivity of the sulfide-ion is somewhat more tardy, for example a polysulfide, or a sulfo-salt. Thus it is possible, for instance, to develop the latent image in a layer containing the salt  $(Co(NH_3)_5(NO_2)_2C_2O_4)NH_4$  as sensitive substance, by means of a sodium polysulfide solution. The following experiment shows that this is actually a development, not merely a conversion of the light-decomposition product into sulfide. If one writes on a pure gelatine layer with a cobalt chloride solution of 0.001 per cent strength, the written characters cannot be rendered visible by a subsequent treatment with a sodium-polysulfide solution in consequence of the excessively small concentration of cobalt salt; if, however, the gelatine layer contains from the outset some of the complex salt of the above formula the writing in cobalt chloride becomes very prominent on treatment with sodium polysulfide as in this case the extremely small quantity of cobalt chloride determines formation of cobalt sulfide from the complex compound.

The process is not limited to the above-mentioned cobalt complex salt, but for the purpose there is suitable a very large number of compounds which on the one hand are sufficiently sensitive to light and on the other hand yield dark sulfides, such as nickel, iron, copper or like compounds.

As already briefly explained above, suitable developers are principally sulfides which in consequence of formation of polysulfide or sulfo-salt are less reactive than pure sulfides. As developers there may also be used mixtures of substances which react only relatively slowly with the formation of free sulfide-ion, such as, for example, a solution of thioacetamide and caustic soda solution.

The light-sensitive substances which come under consideration are further characterized in that in a number of them the latent image, which can be developed, can be produced not only by the energy of the light rays, but, for instance, with nickel complex compounds by that of heat rays or, for instance, with lead compounds by that of X-rays or by that of electric currents.

25 The following examples illustrate the invention:

*Example 1.*—30 cc. of a lead nitrate solution of 10 per cent strength are mixed with 10 cc. of gum arabic solution (10 per cent) and the mixture is precipitated by adding 33 cc. of potassium iodide solution of 10 per cent strength. To the very fine suspension alcohol is added, and the settled precipitate is washed several times with alcohol containing water and then freed as far as possible from alcohol by filtration. The residue on the filter is dissolved in 50 cc. of water and mixed with 100 cc. of gelatine solution of 10 per cent strength, 1 gram of thioacetamide and 10 cc. of glycerine. The finished emulsion is cast in known manner. Thus a very highly light-sensitive material is obtained which also reacts to Röntgen-rays whose latent image can be developed by the following developer

|                  |          |       |
|------------------|----------|-------|
| H <sub>2</sub> O | cc...    | 1,000 |
| Thioacetamide    | grams... | 10    |
| NaOH             | grams... | 3     |

The time of developing amounts to about 1 to 3 minutes. After the development, the picture is preferably treated with a dilute sodium thiosulfate solution.

*Example 2.*—2 grams of (Co(NH<sub>3</sub>)<sub>2</sub>(NO<sub>2</sub>)<sub>4</sub>)NH<sub>4</sub> which has been purified by recrystallizing several times very carefully, are dissolved in 100 cc. of water and, at a maximum temperature of 40° C., are mixed with 50 cc. of gelatine solution of 10 per cent strength. A latent image can be produced in a layer obtained from this solution by light or by an electric current. The latent image is developed by a solution of the following composition:

In a solution of 5 grams of ammonium sulfide in 100 cc. of water, 1 gram of sulfur is dissolved by boiling. For use, this solution is diluted with 10 times its volume of water.

65 The duration of development amounts to 1 to 2 minutes; the picture is fixed by washing with water. In this manner deep brown pictures are obtained.

70 What I claim is:

1. A process of producing photographic pictures which comprises exposing to light an emulsion layer containing a compound of a heavy metal capable of forming a dark-colored sul-

fide until developable nuclei are formed, and treating the latent image thus produced with a solution containing a thio-compound capable of forming the metal sulfide to form a visible image from the latent image immediately following exposure.

2. A process of producing photographic pictures which comprises exposing to light an emulsion layer containing a complex compound of a heavy metal, said complex compound being capable to form under the action of light a compound which contains the metal in ionizable linkage until developable nuclei are formed, and treating the latent image thus obtained with a solution containing a thio-compound capable of forming the metal sulfide to form a visible image from the latent image immediately following exposure.

3. A process of producing photographic pictures which comprises exposing to light an emulsion layer containing a compound of a heavy metal selected from the group consisting of lead, copper, bismuth, silver, mercury, thallium, molybdenum, tungsten, uranium, cobalt and nickel until developable nuclei are formed, and treating the latent image thus produced with a solution containing a thio-compound capable of forming the metal sulfide to form a visible image from the latent image immediately following exposure.

4. A process of producing photographic pictures which comprises exposing to light an emulsion layer containing a complex compound of a heavy metal selected from the group consisting of cobalt, nickel and copper with a compound selected from the group consisting of nitrates, oxalates, amines and phenolates until developable nuclei are formed, and treating the latent image thus formed with a solution containing a thio-compound capable of forming the metal sulfide to form a visible image from the latent image immediately following exposure.

5. A process of producing photographic pictures which comprises exposing to light an emulsion layer containing (Co(NH<sub>3</sub>)<sub>2</sub>(NO<sub>2</sub>)<sub>4</sub>)NH<sub>4</sub> until developable nuclei are formed and treating the latent image thus obtained in an aqueous solution of ammonium-polysulfide to form a visible image from the latent image immediately following exposure.

6. A process of producing photographic pictures which comprises exposing to light an emulsion layer containing a compound of a heavy metal capable of forming a dark-colored sulfide and a thio-compound capable of forming the metal-sulfide, until developable nuclei are formed, and treating the latent image thus produced with a solution containing a thio-compound capable of forming the metal-sulfide, to form a visible image from the latent image immediately following exposure.

7. A process of producing photographic pictures which comprises exposing to light an emulsion layer containing a compound of a heavy metal selected from the group consisting of lead, copper, bismuth, silver, mercury, thallium, molybdenum, tungsten, uranium, cobalt and nickel and a thio-compound capable of forming the metal-sulfide, until developable nuclei are formed, and treating the latent image thus produced with a solution containing a thio-compound capable of forming the metal sulfide to form a visible image from the latent image following exposure.